# EUROPEAN PATENT SPECIFICATION

(11) **EP 0 156 536 B1**
(45) Date of publication and mention of the grant of the patent: **04.07.1990**
(21) Application number: 85301438.9
(22) Date of filing: 01.03.1985
(51) Int. Cl.: E04D 5/12

(54) **Spliceable sheet material and transfer tape for use in making same**
Schweissbare Membran und Übertragungsband zum Gebrauch bei der Herstellung derselben
Membrane soudable et ruban de transmission à utiliser dans sa fabrication

(30) Priority: 23.03.1984 US 592620; 23.03.1984 US 592711
(43) Date of publication of application: 02.10.1985
(73) Proprietor: MINNESOTA MINING AND MANUFACTURING COMPANY, St. Paul, Minnesota 55133-3427 (US)
(72) Inventor: Levens, Dennis L. c/o Minnesota Mining and, St. Paul Minnesota 55133-3427 (US); Renstrom, Richard L. c/o Minnesota Mining and, St. Paul Minnesota 55133-3427 (US)
(74) Representative: Baillie, Iain Cameron

(56) References cited:
- DE-A- 2 752 490
- FR-A- 1 511 612
- GB-A- 865 806
- GB-A- 1 229 292
- GB-A- 1 382 826
- US-A- 1 848 076
- US-A- 3 650 870

## Description

### Background of the Invention

This invention relates to the sealing of overlapped rubbery olefinic polymer (i.e., homopolymer, copolymer, terpolymer, etc.) sheets to each other, to spliceable sheets, to a method of making such sheets, and to the fabrication of a roof covering using such sheets.

Rubbery olefinic polymer sheet material finds widespread industrial use in applications where it is necessary to contain or exclude liquids. Compared to vinyl sheet material, the rubbery olefinic polymer sheet materials have longer life, greater flexibility and resilience at low temperatures, ability to withstand high temperatures without stretching or softening unduly, and superior resistance to ultraviolet light. The most widely used rubbers for formulating these sheets are polymers of ethylene, propylene, and diene monomers (commonly known as EPDM), butyl rubber, and blends of the two. In making rubbery sheet material, the olefinic polymers are commonly blended with desired fillers, coloring agents, extenders, vulcanizing or crosslinking agents, antioxidants, etc. to form a "compound", which is then calendered or extruded into sheets (commonly known as "membranes"), typically on the order of 1.5 millimeters thick and 2 to 6 meters wide. These membranes are then heated to perhaps 150°C. for 2 hours to effect vulcanization.

For many of the applications in which rubbery membranes are employed, it is necessary to overlap and splice the edges of a large number of sheets. Rubbers, which have low energy surfaces, are unreceptive to many adhesives. Accordingly the splicing procedure has heretofore typically involved the steps of cleaning the overlapped areas, applying a primer solution to each face, allowing the solvent to evaporate, applying a contact adhesive solution to each face, again allowing the solvent to evaporate to leave a tacky adhesive surface, mating the contact adhesive-coated surfaces, and compacting the spliced area with a heavy steel roller. Operating in this way, it is possible to form extremely large spliced membranes which can be used to line water reservoirs, irrigation canals, sewage lagoons, industrial waste pits, and solar energy ponds; such products are popularly designated "geomembranes". The splicing process is, however, extremely labor- intensive and costly.

Another important application for spliced rubbery membranes is in the installation of flat roofs for commercial, institutional, and industrial buildings. Spliced membranes are laid over new or existing roofs and typically either fastened down (e.g., at 40-centimeter intervals) with metal battens or ballasted with round river-washed stones. When employed on a roof, extremely rigorous demands are placed on the rubbery membranes, particularly on the splices. Roof temperatures may approach the boiling point of water when exposed to the summer sun, and they may sink to -30°C. - or even lower- during the winter.

In all of the applications for spliced membranes just described, the splicing has been a tedious and time-consuming part of fabrication. How to simplify the preparation of lapped splices has remained an unsolved problem.

US-A-3,650,874 discloses heat-sealable rubber products e.g. rubberised fabric, which are coated with a thin layer of polyolefin, the polyolefin having a melt index of less than 0.15 "when measured according to the standard ASTM 1238-57T modified by adding a supplementary load of 3 kg". It is taught that only low melt-index polyolefins can be adhered to rubber. Furthermore, it is taught that a layer of high melt-index polyolefin can be indirectly adhered to the rubber by sealing it to the coating of low melt-index polyolefin on the surface of the rubber.

DE-A-2,752,490 discloses a composite roofing membrane comprising a lower thermoplastic sheet having a softening point between 100° and 200°C and a protective rubber sheet laid on top of the thermoplastic sheet so as to leave a border area of the thermoplastic sheet exposed. This border area can be heat-sealed to the edge portion of the thermoplastic sheet of a similar composite roofing membrane to form a lapped seam. However, the protective rubber sheet of the disclosed roofing membrane is not firmly bonded to the polyolefin sheet and it is stated that "the limited adhesive strength between the upper and the lower layers also has the advantage, that strips of the upper layer may be separated from the composite sheet during the installation of the roofing sheets".

GB-A-1,382,826 discloses a spliceable sheet material suitable for use in the fabrication of lapped-seam membrane roofing, comprising in combination: a rubbery water-impermeable membrane consisting essentially of thermoset elastomeric olefin polymer, said membrane having on one side, at least in a border area along one edge, an adhesive layer of heat-sealable polyolefin that is capable of wetting the thermoset olefin polymer, and is firmly bonded thereto.

### Brief Description of the Invention

The present invention provides a spliceable sheet material as disclosed in GB-A-1,382,826 characterised in that said heat-sealable polyolefin has a softening point of at least 120°C, and a melt index of 0.5 or greater.

When such sheets are heat-sealed, the resultant splices are strong, resistant to temperature extremes, and able to withstand the expansion and contraction that results from exposure to summer and winter conditions, all the while maintaining a water-tight seal.

The invention also provides a method of making the above sheet material, comprising applying said adhesive layer to an uncured sheet of elastomeric olefin polymer, and then applying heat and pressure to the resulting assembly sufficient to cure the elastomeric olefin polymer and simultaneously bond the adhesive layer thereto.

Preferably, the adhesive layer of heat-sealable polyolefin is a thin layer e.g. of thickness 90 urn. Further preferred embodiments are claimed in the dependent claims.

A presently preferred material for the rubbery olefin polymer membrane is EPDM, and a presently preferred adhesive is linear low density polyethylene having a softening point (as defined in ASTM Test D-16, Procedure 19) of at least 120°C. (It should be recognized that the term "polyethylene" may include the normally employed stabilizers, filers, extenders, processing aids, pigments, and the like.) Other suitable adhesives can be formulated from thermoplastic blends of polyethylene and polypropylene, homopolymers of olefin monomers, polymers of two or more olefin monomers, etc., provided that the softening point meets the stated temperature requirement. To enhance processability, the melt index of the adhesive is desirably at least 0.5 a melt index of about 1 being presently preferred. For convenience in use, preferably the softening point of the heat-sealable adhesive should not exceed 250°C., and preferably is significantly lower, to minimize the possibility of degrading the rubbery membrane.

A presently preferred spliceable sheet material of the type described in the preceding paragraph is one in which linear low density polyethylene is adhered to the border area on one side of the rubbery sheet material adjacent a lateral edge and also on the border area on the other side adjacent the opposite lateral edge, this arrangement lending itself to a natural shingling type of overlapping.

A simple but unique transfer tape having particular utility in making the spliceable border areas of the sheet material just described comprises a release liner having strippably adhered to one face a thin layer of heat-sealable adhesive. A preferred transfer tape construction comprises a polyester film release liner, e.g., biaxially oriented polyethylene terephthalate, carrying a heat-sealable thermoplastic polyolefin layer, e.g., linear low density polyethylene. Spliceable rubbery sheet material may then conveniently be fabricated by placing the adhesive surface of the transfer tape in contact with the appropriate area or areas of the rubbery membrane and applying sufficient heat and pressure to melt the adhesive and bond it to the membrane. A particularly preferred method is to place the transfer tape in contact with the unvulcanized sheet material, apply sufficient pressure to maintain intimate contact between the tape material and heat the assembly to a temperature high enough to vulcanize (i.e., crosslink, or thermoset) the olefin polymer and, at the same time, soften the adhesive, thereby permitting it to wet and upon cooling, bond firmly to the olefinic polymer sheet. The release liner may then remain in place to protect the adhesive from contamination and be removed at the time a splice is to be made.

The sheet material of the invention may be used to form a roof covering by a method as claimed in claim 14.

Because it is difficult, expensive, and time-consuming to conduct field evaluations of products made in accordance with the invention, a number of tests have been developed to provide information that relates directly to some aspect of roofing end use requirements. These tests, which incorporate built-in safety factors, are briefly described below.
1. T-Peel Test. In this test, two 2.54-cm wide x 15-cm long x 1.14-mm thick strips of commercially available EPDM-based membrane, each provided with a 38-micrometer layer of heat-activatable adhesive, are superposed in coextensive adhesive-to-adhesive contact and approximately 5 cm at one end laminated for one minute in a press at 160°C. and 20 kPa. Conventional T-peel tests are then performed in tensile testing equipment in which the jaws are separated at a rate of 30.5 cm/minute. For roofing applications, initial values should be at least 8.8 N/cm when tested at room temperature. After being subjected to any one of the conditions described below and then re-tested, T-peel values should be at least 17.5 N/cm.
   a. Temperature Cycling. T-peel samples are exposed to room temperature for one week, -18°C. for one week, room temperature for another week, -18°C. for one week, and then tested.
   b. Hot Water Immersion. Two hours after being prepared, T-peel samples are immersed for 24 hours in 70°C. water, removed, dried, and tested at room temperature.
   c. Delayed Hot Water Immersion. 24 hours after being prepared, the T-peel samples are immersed in 70°C. water for 24 hours, removed, and tested as in sub-paragraph "b".
   d. High Humidity. T-peel samples are exposed to 38°C. and 100% relative humidity for one week, removed, dried, and tested at room temperature.
   e. Heat Aging. Samples are placed in a 70°C. oven for one week, removed, and tested at room temperature.
   f. Heat Resistance. T-peel samples are heated as in sub-paragraph "e" but tested at 70°C.
   g. Weather Resistance. Samples are exposed to the artificial weathering conditions provided by a "Weatherometer" machine in accordance with ASTM Test D-750. Tests are performed after 250 and 500 hours.
   h. Freeze- Thaw Resistance. T-peel samples are immersed in room temperature water for one week and then placed in a -18°C. freezer for one week. They are removed and tested at room temperature.
2. Softening Point. Strips of the heat-sealable roofing membrane 2.54 cm wide are overlapped 2.54 cm adjacent one end of each and bonded for one minute, adhesive-to-adhesive, in a 160°C. press at a pressure of 20 kPa. The spliced strip is then removed and tested in accordance with a modified form of ASTM-D816 Procedure 19. In this test, the end of one strip is gripped between the jaws of a holder, the remainder of the spliced strip extending vertically, with a 2.27-kg weight attached to the free end. The assembly is then placed in a 65°C. oven and the temperature raised 0.5°C./minute until failure occurs; the acceptable threshold temperature is 120°C.
3. Dynamic Shear. Samples, prepared as in the softening point test, are mounted in a tensile testing machine, the jaws of which are separated at the rate of 1.3 mm/minute until failure occurs. A force of 275 kPa or more is considered acceptable.
4. Static Shear. Lap-spliced samples are prepared as in the preceding two tests. One end of the spliced sample is gripped in the jaws of a holder, with the remainder of the sample extending vertically. To the free end is then attached a 2.27-kg weight and the assembly placed in an 82°C. oven. Failure should not occur in less than 24 hours.
5. Low Temperature Flexibility. Two 2.54 cm x 12.5 cm strips of heat-sealable roofing membrane are superposed in adhesive-to-adhesive contact and bonded in a 160°C. press under a pressure of 20 kPa for one minute. The resulting laminate is conditioned in a freezer maintained at -34°C. for 24 hours. An operator, wearing gloves to avoid heating the samples, then bends the sample around a 1.27-cm. diameter refrigerated steel rod, removes it, and bends it in the opposite direction around the rod, repeating the cycle five times. No evidence of delamination should occur.

### Detailed Description

The invention will now be described with the aid of illustrative but non-limiting examples, in which all parts and percentages are by weight unless otherwise indicated.

### Example 1

A linear low density polyethylene (Union Carbide "G-Resin 7047 Natural 7"), having a melt index of 1.0, was extruded through a slot die having an opening of 0.56 mm at a die head temperature of 250°C. Immediately after emerging from the die, the extruded polyethylene film was contacted by a 38- micrometer polyester film; the resulting laminate was pulled between a rubber roll and metal roll, located approximately 75 mm from the die opening. The rolls were driven at a considerably faster surface speed than the rate at which the polyethylene was extruded, so that the polyethylene thickness was reduced to approximately 90 micrometers. Samples approximately 75 mm x 100 mm were then cut from the laminate and used for further testing. The polyethylene was tack-free at room temperature.

A sample of the laminate was positioned with the polyethylene layer against a smooth sheet of 1.5-mm cured EPDM rubber, and placed for 30 seconds in a press heated to 218°C. under a pressure of approximately 35 kPa. The sample was then removed from the press and allowed to cool to room temperature, after which the polyester release liner was stripped away, exposing the heat-sealable polyethylene surface. The stripping force required was about 0.03 N/cm width. Values of at least about 0.02 N/cm are desirable for ease in processing, values somewhat in excess of 0.1 N/cm being satisfactory but not preferred. Significantly higher stripping values make the product more difficult for the end user to remove the release liner.

### Example 2

A polyethylene-polypropylene blend (Eastman Chemical Company "Tenite" 5321E polyallomer) was extruded through a 0.38-mm 240°C. die head and processed as in Example 1.

The adhesive-coated EPDM products made in accordance with the preceding examples were then tested in accordance with the previously described procedures. Results are tabulated below:

In factory production operations, it has been found convenient to apply the linered heat-sealable adhesive directly to the uncured EPDM rubber membrane in 5.0-7.5-cm strips along the border of one side adjacent the edge. The assembly is then subjected to 375 kPa pressure at 150°C. to cure the EPDM rubber and simultaneously bond the heat-sealable adhesive firmly thereto. Workers in the field lay out the rubber membrane in a manner such that the heat-sealable portion of one strip of material overlaps the edge of an adjacent strip of material, after which they remove the liner. Heat is then applied, either directly to the adhesive or to the opposite side of the adhesive-bearing rubber membrane in the splice area, to soften the adhesive and cause it to bond firmly to the underlying edge of the adjacent strip.

In circumstances where the rubber membrane has an embossed or irregular surface, adhesion in the splice area will be enhanced if confronting border portions of the overlapped strips are both provided with a heat-sealable coating. This construction can be achieved during factory production by making sure that a first heat-sealable transfer tape is positioned on one side adjacent one edge and a second heat-sealable transfer tape is positioned on the other side adjacent the second edge.

In some circumstances, it may be advantageous to coat one entire side of the rubber membrane with heat-sealable coating. With completely coated membranes of this type, rolls of the membrane may be slit to any desired width, e.g., to fit narrow portions of a roof, while still maintaining heat-sealable coating adjacent each edge. Another advantage achieved by overall coating with heat-sealable adhesive is the ability to seal directly to the upper surface of batten strips that have been nailed or otherwise affixed to the roof substrate, thereby permitting completely imperforate roofing membrane construction. For such purposes, it is advantageous to use batten strips made of polyethylene, which are not only moisture- and rust-resistant but also inherently possess heat-sealable properties and are compatible with the thermoplastic olefinic heat-sealable coating on the roofing membrane. If, of course, the polyethylene batten strips are used only in the spliced areas, it is adequate to have heat-sealable adhesive only in the border area of the lower membrane, where it will contact the batten strip.

It will be appreciated that varying the composition of the rubber membrane may make it desirable to modify the heat-sealable adhesive composition. Also, as indicated earlier in the discussion of this invention, the performance requirements for roof construction are somewhat more strenuous than may be required for such other applications as pond or swimming pool liners; for such uses, other heat-sealable adhesives should be able to perform effectively. Those skilled in the art will, however, have no difficulty in determining suitable adhesives to be employed in appropriate circumstances, considering the foregoing discussion.

## Claims

1. A spliceable sheet material suitable for use in the fabrication of lapped-seam membrane roofing, comprising in combination: a rubbery water-impermeable membrane consisting essentially of thermoset elastomeric olefin polymer, said membrane having on one side, at least in a border area along one edge, an adhesive layer of heat-sealable polyolefin that is capable of wetting the thermoset olefin polymer, and is firmly bonded thereto, characterised in that said heat-sealable polyolefin has a softening point of at least 120°C, and a melt index of 0.5 or greater.

2. A strip of sheet material as claimed in claim 1, wherein said adhesive layer is confined to a border area adjacent a side edge of the strip.

3. A strip of sheet material as claimed in claim 2 wherein two such adhesive layers are provided, one confined to one border area adjacent one side edge of the strip, and the other being confined to another border area adjacent the opposite side edge of the strip on the opposite face of the strip.

4. A roll of sheet material as claimed in claim 1.

5. Sheet material as claimed in any preceding claim wherein said adhesive layer has a thickness of approximately 90 pm.

6. Sheet material as claimed in any preceding claim wherein the olefin polymer consists essentially of polymerized ethylene, propylene, and diene monomers (EPDM).

7. Sheet material as claimed in any preceding claim wherein said adhesive is an olefin homopolymer.

8. Sheet material as claimed in claim 6 wherein the heat-sealable adhesive is linear low density polyethylene having a melt index of about 1.0.

9. Sheet material as claimed in any preceding claim wherein the heat-sealable adhesive is protectively covered by a strippable liner.

10. Sheet material as claimed in claim 9 wherein the release liner is a film of biaxially oriented polyethylene terephthalate.

11. Sheet material as claimed in claim 6 wherein said adhesive is a blend of polyethylene and polypropylene.

12. A method of making sheet material as claimed in any of claims 1 to 8 and 11, comprising applying said adhesive layer to an uncured sheet of elastomeric olefin polymer, and then applying heat and pressure to the resulting assembly sufficient to cure the elastomeric olefin polymer and simultaneously bond the adhesive layer thereto.

13. A method of making sheet material as claimed in claim 9 or claim 10 comprising the steps of:
a. obtaining an uncured but curable sheet of polyolefinic compound,
b. placing in contact with a lateral border on one side of said sheet a transfer tape comprising a thermoplastic olefinic layer carried by a strippable release liner, the olefinic layer of the tape having a softening point of at least 120°C and a melt index of at least 0.5, and being in contact with said sheet, to form an assembly,
c. subjecting said assembly to elevated pressure and temperature for a time sufficient to cure said compound and firmly bond the heat-sealable thermoplastic olefinic layer to the cured sheet material.

14. A method of forming a roof covering comprising the steps of laying a sheet of material as claimed in any of claims 1 to 10 on a roof, laying a further sheet of material as claimed in any of claims 1 to 10 such that the adhesive layer of one of said sheets is superimposed on the other of said sheets, heating the adhesive layer to form a bond between the sheets, and repeating said steps with further such sheets as necessary to form said roof covering.

15. A method as claimed in claim 14, wherein said sheets are laid over, and adhered to, plastic batten strips previously affixed on the roof substrate.

16. A composite membrane comprising two or more sheets of sheet material as claimed in any of claims 1 to 11 bonded together by a said adhesive layer in an overlapping relationship.

17. A composite membrane as claimed in claim 16 which is a roofing membrane.

## Revendications

1. Matériau en feuille soudable convenant pour l'utilisation dans la fabrication de couverture de toit à membranes jointes en recouvrement, comprenant en combinaison: une membrane caoutchouteuse imperméable à l'eau, constituée essentiellement d'un polymère d'oléfine élastomère thermodurci, ladite membrane comportant sur une face, au moins dans une région de bordure le long d'un bord, une couche adhésive de polyoléfine thermosoudable qui est capable de mouiller le polymère d'oléfine thermodurci et est liée solidement à celui-ci, caractérisé en ce que ladite polyoléfine thermosoudable a un point de ramollissement d'au moins 120°C, et un indice d'écoulement à l'état fondu de 0,5 ou plus.

2. Bande de matériau en feuille suivant la revendication 1, dans laquelle ladite couche est limitée à une région de bordure adjacente à un bord latéral de la bande.

3. Bande de matériau en feuille suivant la revendication 2, dans laquelle il est prévu deux telles couches adhésives, l'une étant limitée à une région de bordure adjacente à un bord latéral de la bande, et l'autre étant limitée à une autre région de bordure adjacente au bord latéral opposé de la bande sur la face opposée de la bande.

4. Rouleau de matériau en feuille suivant la revendicaiton 1.

5. Matériau en feuille suivant l'une quelconque des revendications précédentes, dans lequel ladite couche adhésive a une épaisseur de 90 pm environ.

6. Matériau en feuille suivant l'une quelconque des revendications précédentes, dans lequel le polymère d'oléfine est constitué essentiellement de monomère d'éthylène, de propylène et de diènes polymérisés (EPDM).

7. Matériau en feuille suivant l'une quelconque des revendications précédentes, dans lequel ledit adhésif est un homopolymère d'oléfine.

8. Matériau en feuille suivant la revendication 6, dans lequel l'adhésif thermosoudable est du polyéthylène linéaire basse densité ayant un indice d'écoulement à l'état fondu de 1,0 environ.

9. Matériau en feuille suivant l'une quelconque des revendications précédentes, dans lequel l'adhésif thermosoudable est recouvert d'une doublure de protection séparable.

10. Matériau en feuille suivant la revendication 9, dans lequel la doublure séparable est un film de téréphtalate de polyéthylène orienté biaxialement.

11. Matériau en feuille suivant la revendication 6, dans lequel ledit adhésif est un mélange de polyéthylène et de polypropylène.

12. Procédé de fabrication d'un matériau en feuille suivant l'une quelconque des revendications 1 à 8 et 11, comprenant l'application de ladite couche adhésive à une feuille non durcie de polymère d'oléfine élastomère, puis l'application de chaleur et de pression à l'assemblage résultant, suffisamment pour durcir le polymère d'oléfine élastomère et lier simultanément la couche adhésive à celui-ci.

13. Procédé de fabrication d'un matériau en feuille suivant la revendication 9 ou la revendication 10, comprenant les opérations de:
a. préparation d'une feuille non durcie mais durcissable de composé polyoléfinique,
b. mise en contact, avec une bordure latérale sur une face de ladite feuille, d'un ruban de transfert comprenant une couche oléfinique thermoplastique portée par une doublure de protection décollable, la couche oléfinique du ruban ayant un point de ramollissement d'au moins 120°C et un indice d'écoulement à l'état fondu d'au moins 0,5, et étant en contact avec ladite feuille, pour constituer un ensemble, et
c. soumission dudit ensemble à une pression et une température élevées pendant un temps suffisant pour durcir ledit composé et lier solidement la couche oléfinique thermoplastique thermosoudable au matériau en feuille durci.

14. Procédé de formation d'une couverture de toit, comprenant les opérations de pose d'une feuille de matériau suivant l'une quelconque des revendications 1 à 10 sur un toit, de pose d'une autre feuille de matériau suivant l'une quelconque des revendications 1 à 10, de sorte que la couche adhésive d'une desdites feuilles soit superposée à l'autre desdites feuilles, de chauffage de la couche adhésive pour engendrer une liaison entre les feuilles, et de répétition desdites opérations avec d'autres feuilles semblables, comme nécessaire pour former ladite couverture de toit.

15. Procédé suivant la revendication 14, dans lequel lesdites feuilles sont posées et collées sur des lattes en matière plastique préalablement fixées au substrat du toit.

16. Membrane composite comprenant deux feuilles et plus de matériau en feuille suivant l'une quelconque des revendications 1 à 11, liées les unes aux autres par une dite couche adhésive en relation de chevauchement.

17. Membrane composite suivant la revendication 16, qui est une membrane de couverture de toit.

## Patentansprüche

1. Spleißbares Blattmaterial, das für die Verwendung bei der Herstellung von Membrandachbelag mit Überlappfugen geeignet ist, umfassend, im Kombination: eine gummiartige, wasserundurchlässige Membran, die im wesentlichen aus einem duroplastischen elastomeren Olefinpolymer besteht und die auf einer Seite mindestens im Bereich eines Randes mit einer Klebstoffschicht aus einem heißsiegelbaren Polyolefin versehen ist, das zum Benetzen des duroplastischen Olefinpolymers befähigt und stoffschlüssig fest damit verbunden ist, dadurch gekennzeichnet, daß das heißsiegelbare Polyolefin einen Erweichungspunkt von mindestens 120°C und einen Schmelzindex von 0,5 oder mehr hat.

2. Band aus einem Blattmaterial nach Anspruch 1, dadurch gekennzeichnet, daß die Klebstoffschicht nur im Bereich eines Seitenrandes des Streifens vorgesehen ist.

3. Band aus einem Blattmaterial nach Anspruch 2, dadurch gekennzeichnet, daß zwei derartige Klebstoffschichten vorgesehen sind, von denen die eine nur im Bereich eines Seitenrandes des Bandes und die andere nur auf der entgegengesetzten Fläche des Bandes im Bereich des entgegengesetzten Seitenrandes des Bandes vorgesehen ist.

4. Rolle aus Blattmaterial nach Anspruch 1.

5. Blattmaterial nach einem der vorhergehenden Ansprüche, dadurch gekennzeichnet, daß die Klebstoffschicht eine Dicke von etwa 90 um hat.

6. Blattmaterial nach einem der vorhergehenden Ansprüche, dadurch das Olefinpolymer im wesentlichen aus polymerisiertem Monomeren des Ethylens, Propylens und Diens (EPDM) besteht.

7. Blattmaterial nach einem der vorhergehenden Ansprüche, dadurch gekennzeichnet, daß der Klebstoff ein Olefinhomopolymer ist.

8. Blattmaterial nach Anspruch 6, dadurch gekennzeichnet, daß der heißsiegelbare Klebstoff ein lineares Polyethylen von geringer Dichte und mit einem Schmelzindex von ungefähr 1,0 ist.

9. Blattmaterial nach einem der vorhergehenden Ansprüche, dadurch gekennzeichnet, daß der heißsiegelbare Klebstoff mit einer abziehbaren Abdeckung geschützt ist.

10. Blattmaterial nach Anspruch 9, dadurch gekennzeichnet, daß die Antihaftabdeckung aus einer Folie aus biaxial orientiertem Polyethylenterephthalat besteht.

11. Blattmaterial nach Anspruch 6, dadurch gekennzeichnet, daß der Klebstoff ein Gemisch aus Polyethylen und Polypropylen ist.

12. Verfahren zum Herstellen von Blattmaterial nach einem der Ansprüche 1 bis 8 und 11, in dem die Klebstoffschicht auf ein ungehärtetes Blatt aus einem elastomeren Olefinpolymer aufgetragen und die so erhaltene Anordnung der Einwirkung von Wärme und Druck in einem solchen Maße unterworfen wird, daß das elastomere Olefinpolymer gehärtet und gleichzeitig die Klebstoffschicht stoffschlüssig damit verbunden wird.

13. Verfahren zum Herstellen von Blattmaterial nach Anspruch 9 oder 10 mit folgenden Schritten:
a. es wird en ungehärtetes, aber härtbares Blatt aus einer polyolefinischen Verbindung beschafft,
b. ein Übertragungsband mit einer thermoplastischen olefinischen Schicht auf einer abziehbaren Antihaftauflage wird mit einem Randbereich auf einer Seite des Blattes in Berührung gebracht, wobei die olefinische Schicht des Bandes einen Erweichungspunkt von mindestens 120°C und einen Schmelzindex von mindestens 0,5 hat und mit dem Blatt in Berührung steht, so daß eine Anordnung erhalten wird,
c. diese Anordnung wird solange einem erhöhten Druck und einer erhöhten Temperatur unterworfen, daß die genannte Verbindung gehärtet und die heißsiegelbare thermoplastische olefinische Schicht mit dem gehärteten Blattmaterial fest stoffschlüssig verbunden wird.

14. Verfahren zum Herstellen eines Dachbelages mit folgenden Schritten: ein Blatt aus einem Material nach einem der Ansprüche 1 bis 10 wird auf ein Dach gelegt, ein weiteres Blatt aus einem Material nach einem der Ansprüche 1 bis 10 wird so gelegt, daß die Klebstoffschicht eines der Blätter auf dem anderen Blatt liegt, durch Erhitzen der Klebstoffschicht werden die Blätter stoffschlüssig miteinander verbunden, und diese Schritte werden mit weiteren derartigen Blättern wiederholt, soweit es zur Bildung des Dachbelages notwendig ist.

15. Verfahren nach Anspruch 14, dadurch gekennzeichnet, daß die genannten Blätter auf Fugendeckleisten aus Kunststoff gelegt und mit ihnen verklebt werden, die vorher auf der Dachunterlage befestigt worden sind.

16. Verbundmembran mit zwei oder mehreren Blättern aus einem Blattmaterial nach einem der Ansprüche 1 bis 11, wobei diese Blätter einander überlappend durch die Klebstoffschicht formschlüssig miteinander verbunden sind.

17. Verbundmembran nach Anspruch 16, die eine Dachbelagmembran ist.
